

# UNITED STATES PATENT OFFICE.

WILLIAM R. D. HALL, OF NARBERTH, PENNSYLVANIA.

## PROCESS FOR TREATING ARTIFICIAL-SILK WASTE FOR SPINNING INTO YARN.

1,303,301.

Specification of Letters Patent. Patented May 13, 1919.

No Drawing.

Application filed June 26, 1918. Serial No. 242,110.

*To all whom it may concern:*

Be it known that I, WILLIAM R. D. HALL, a citizen of the United States, residing at Narberth, in the county of Montgomery and 5 State of Pennsylvania, have invented new and useful Improvements in Processes for Treating Artificial-Silk Waste for Spinning into Yarn, of which the following is a specification.

10 This invention aims to produce a process by which artificial silk waste may be treated so as to satisfactorily spin the same into yarn.

I have found that when the moisture content of the silk waste is above 8 per cent. the absorption in artificial silk waste is most complete and causes the material to become too weak, resulting in a short staple.

On the other hand, when the moisture content is below 6 per cent. the material becomes too brittle to be worked, *i. e.*, when the same is to be turned into yarn the waste breaks and is consequently not of sufficient length to produce a yarn of uniform smoothness 25 and firmness, resulting in the same disadvantage caused when the moisture content of the waste is below 6 per cent.

It will thus be seen that it is very difficult to produce a yarn from silk waste, of the 30 artificial kind, of uniform quality and smoothness as it will be readily appreciated that it is almost impossible to keep the moisture content between 6 and 8 per cent. in such waste, and I have therefore conceived 35 the following idea whereby the constant moisture content of between 6 and 8 per cent. in artificial silk waste which is about to be made up into yarn is insured.

An air-tight room is provided in which the 40 artificial silk waste is placed, which room has a moisture content of the desired quality, *i. e.*, from 6 to 8 per cent. Consequently, the waste absorbs the needed moisture content or evaporates any extra moisture which it may 45 contain and after remaining in this room for a certain time, the same is in a condition to be worked.

However, it will be readily appreciated that in such a fine fiber as that of artificial 50 silk the moisture content would be varied no matter how quickly the waste might be removed from the conditioning room to the machine. In order to guard against this and to keep the moisture content of the waste 55 as it was at the time of leaving the conditioning room, I apply to the same lard oil

in the proportion of  $6\frac{1}{2}$  per cent. of the weight of the conditioned material or to the same, before its removal from the conditioning room. This oil effectively guards 60 against any evaporation or absorption of moisture by the material.

It will be seen that by the above process I have overcome the aforementioned objections to the working of artificial silk waste 65 into yarn or other purposes.

Having described my invention, what I claim is:—

1. The process of conditioning artificial silk waste so that it may have its proper 70 moisture content, which consists in placing the same in a conditioning room having its atmosphere charged with the proper moisture content and in then allowing the artificial silk waste to remain in such room until 75 it has either absorbed or evaporated sufficient moisture to have the correct moisture content, and prior to its removal from such room in treating the silk waste with a substance whereby to prevent the loss or absorption 80 of moisture from the air outside of such room.

2. The process of conditioning artificial silk waste so that it may have its proper 85 moisture content, which consists in placing the same in a conditioning room having its atmosphere charged with the proper moisture content and in then allowing the artificial silk waste to remain in such room until 90 it has either absorbed or evaporated sufficient moisture to have the correct moisture content, and in treating such silk waste with an animal oil to prevent its losing or absorbing any moisture subsequent to its removal 95 from such room.

3. The process of conditioning artificial silk waste so that it may have its proper 100 moisture content, which consists in placing the same in a conditioning room having its atmosphere charged with the proper moisture content and in then allowing the artificial silk waste to remain in such room until 105 it has either absorbed or evaporated sufficient moisture to have the correct moisture content, and in applying to such silk waste lard oil, previous to its removal from such room whereby the absorption or evaporation of moisture from such silk waste is prevented after its removal from such room.

4. The process of conditioning artificial 110 silk waste so that it may have its proper moisture content, which consists in placing

the same in a conditioning room having its atmosphere charged with the proper moisture content and in then allowing the artificial silk waste to remain in such room until 5 it has either absorbed or evaporated sufficient moisture to have the correct moisture content, and in applying to such silk waste

lard oil in the proportion of 6½ per cent. previous to its removal from such room whereby the absorption or evaporation of 10 moisture from such silk waste is prevented after its removal from such room.

WILLIAM R. D. HALL.